

## 1

2,905,553

## HIGH STRENGTH ALLOY

Ray W. Guard and Peter J. Clemm, Schenectady, N.Y.,  
assignors to General Electric Company, a corporation  
of New York

No Drawing. Application May 21, 1957  
Serial No. 660,457

4 Claims. (Cl. 75—124)

The present invention relates to alloys which have high strength at temperatures up to and exceeding 1200° F., have improved tensile properties at room temperature, and which may be readily formed into wrought articles as well as sheet stock material having desirable welding properties.

This application is a continuation-in-part of "High Strength Alloy," Serial No. 588,975, filed on June 4, 1956, now abandoned, by the present inventors and assigned to the assignees of this application.

The development of the gas turbine and similar apparatus has created a demand for materials having higher strength and greater stability at elevated temperatures than the high temperature alloys currently available. Certain components of such apparatus such as turbine buckets and blades are subjected to very high stresses over long periods of time in highly corrosive atmospheres at continuous temperatures of the order of 1500° F. or more. Other components such as the turbine wheel members which support the bucket elements, sheet metal members constituting the tail pipe or cone and the like, are similarly subjected to high stresses and corrosive atmospheres at continuous temperatures of the order of 1200° F. or more.

In general, the articles which must withstand the higher stresses and temperatures as noted above, have been fabricated by either precision casting techniques or have been forged from alloys which are capable of being worked to final form from castings or ingots. The workable alloys of this type have usually been precipitation hardenable materials and have usually contained substantial amounts of "strategic" materials such as cobalt and columbium and have usually had as a major constituent, for example, as much as 40 percent or more nickel. These elements are in relatively short supply, are expensive and, further, while these high strength alloys containing these strategic elements are capable of being worked to some degree, they are not readily reducible to sheet material by conventional rolling practices. Furthermore, these materials may be welded only with considerable difficulty and usually exhibit a weakened zone at the weld.

Alloys which have been employed as structural elements at about 1200° F. have been lower in strategic element content and have been more readily workable. These materials have usually been modified stainless steels and have been only moderately weldable. In general, the more easily and successfully weldable materials have had lower mechanical properties such as stress rupture strength and elevated temperature ultimate and yield strengths while those which have had higher mechanical properties, particularly at temperatures of the order of 1200° F. and higher have been more difficult to work and have not been as satisfactorily welded.

## 2

Accordingly, a principal object of our invention is the provision of an alloy having high mechanical strength and resistance to corrosion at elevated temperatures which is readily fabricated by forging or rolling and which is readily welded.

A further object of our invention is the provision of such an alloy which is readily reduced by rolling into sheet metal.

Other and specifically different objects of our invention will become apparent to those skilled in the art from the following disclosure.

Briefly stated, in accordance with one aspect of our invention we provide an austenitic alloy consisting essentially of from about 30.0 to 35.0 percent by weight nickel, from about 12 to about 15 percent chromium, from about 5.5 to 7.5 percent tungsten, from about 2.5 to about 5 percent molybdenum, from about 1.5 to about 4.5 percent titanium, up to about 0.50 percent aluminum, up to about 0.50 percent zirconium, up to about 0.10 percent carbon, and the balance substantially all iron, which alloy has higher mechanical properties than previously obtainable with similarly known materials and which is more readily formed and successfully welded than other alloys having similar mechanical strength.

More specifically, we have discovered that an alloy consisting essentially of about 31.0 to 34.0 weight percent and preferably about 33 percent nickel, about 12.5 to 15.0 percent and preferably about 13 percent chromium, about 6.0 to 7.0 percent and preferably about 6 percent tungsten, about 3.0 to 4.6 percent and preferably about 3.5 percent molybdenum, about 1.75 to about 2.5 percent and preferably about 2.0 percent titanium, about 0.2 to 0.5 percent and preferably about 0.45 percent aluminum, not more than about 0.4 percent and preferably about 0.35 percent zirconium, no more than and preferably less than about 0.08 percent carbon, and the balance substantially all iron, has high tensile strength and ductility, high temperature stress rupture strength and ductility, and is readily formed and welded. It will be understood that the phrase "balance substantially all iron" as used herein includes minor amounts of impurities customarily found in ferrous alloys of this type such as, for example, manganese, silicon, sulfur and phosphorus. It has been found that the total of these particular impurities may constitute as much as about 0.2 weight percent of these alloys without impairing their mechanical properties but preferably should not exceed about 0.05 percent manganese, 0.05 percent silicon, 0.04 percent sulfur, and 0.04 percent phosphorus. Of course, other elements may also be present in very small amounts, as is customary in such materials.

Yet further, we have discovered that substantially the same alloy composition, but one which contains from about 2.5 to 4.5% titanium and particularly from about 3 to 4% titanium, exhibits a higher room temperature tensile strength and yield strength than would be expected when compared with the alloys having the lower titanium content.

We have found that the alloys of our invention are more advantageously prepared by melting and casting the various constituents of these alloys under a vacuum. The cast ingots may then be reduced to either forged bodies such as turbine wheels or bar stock, for example, or may be reduced to sheet stock by conventional forging and rolling procedures. The finished material is then subject to solution and aging heat treatment as will be discussed in more detail subsequently.

By way of example, alloys having the following specific compositions were prepared as stated previously.

Table I

| Heat No. | Ni   | Cr   | W   | Mo  | Ti  | Al   | Zr   | C    | Fe   |
|----------|------|------|-----|-----|-----|------|------|------|------|
| 1        | 32.9 | 13.0 | 6.4 | 3.1 | 2.2 | 0.35 | 0.20 | 0.04 | 42.0 |
| 2        | 32.9 | 13.1 | 6.7 | 3.6 | 1.6 | 0.39 | 0.16 | 0.04 | Bal. |
| 3        | 31.7 | 14.7 | 6.8 | 2.6 | 2.1 | 0.27 | 0.07 | 0.04 | 42.3 |
| 4        | 32.2 | 12.8 | 6.3 | 3.5 | 2.1 | 0.50 | 0.05 | 0.10 | Bal. |
| 5        | 32.5 | 12.8 | 6.2 | 3.5 | 1.9 | 0.39 | 0.17 | 0.04 | Bal. |
| 6        | 32.8 | 12.7 | 6.1 | 3.4 | 2.0 | 0.31 | 0.06 | 0.06 | Bal. |
| 7        | 32.8 | 13.1 | 6.0 | 3.2 | 1.9 | 0.15 | 0.08 | 0.06 | Bal. |
| 8        | 32.2 | 12.8 | 6.0 | 3.6 | 1.9 | 0.34 | 0.10 | 0.04 | Bal. |
| 9        | 32.4 | 13.0 | 3.0 | 3.6 | 1.9 | 0.37 | 0.05 | 0.06 | Bal. |
| 10       | 32.4 | 12.8 | 6.1 | 3.4 | 2.8 | 0.41 | 0.05 | 0.05 | Bal. |
| 11       | 32.5 | 12.9 | 6.1 | 3.4 | 3.8 | 0.43 | 0.16 | 0.06 | Bal. |

Cast ingots from these heats were reduced to round bar stock and to sheet material by conventional forging and rolling procedures. Conventional tensile test and stress rupture test specimens were prepared from this material and heat treated.

Conventional tensile tests were performed on certain of these specimens at room temperature and elevated temperatures. The following data are exemplary of the results of these tests performed on specimens prepared from bar stock.

Table II

| Heat No. | Sol'n Temp. (° F.) | Test Temp. (° F.) | .2% Y.S. (p.s.i.) | Ult. Tens. Str. (p.s.i.) | Percent Elong. (1" g.a.) |
|----------|--------------------|-------------------|-------------------|--------------------------|--------------------------|
| 1        | 2,000              | RT                | 119,000           | 178,000                  | 24.0                     |
|          |                    | 1,350             | 100,000           | 117,000                  | 21.0                     |
|          |                    | RT                | 115,800           | 177,800                  | 23.0                     |
| 2        | 1,900              | 1,200             | 104,200           | 135,500                  | 23.0                     |
|          |                    | 1,350             | 95,400            | 107,500                  | 25.5                     |
|          |                    | RT                | 129,100           | 187,700                  | 18.5                     |
| 3        | 1,850              | 1,200             | 116,800           | 143,900                  | 19.0                     |
|          |                    | 1,350             | 93,100            | 111,400                  | 18.5                     |
|          |                    | RT                | 107,800           | 179,500                  | 23.0                     |
| 4        | 1,850              | 1,200             | 105,000           | 144,100                  | 21.0                     |
|          |                    | 1,350             | 101,400           | 114,800                  | 20.0                     |
|          |                    | RT                | 138,000           | 178,000                  | 17.0                     |
| 5        | 1,850              | 1,350             | 96,000            | 115,000                  | 19.0                     |
|          |                    | RT                | 93,000            | 155,000                  | 17.0                     |
|          |                    | 1,350             | 74,000            | 104,000                  | 15.0                     |
| 6        | 1,850              | 1,350             | 117,000           | 171,000                  | 21.0                     |
|          |                    | RT                | 88,000            | 104,000                  | 15.0                     |
|          |                    | 1,350             | 98,000            | 159,000                  | 20.0                     |
| 7        | 2,150              | 1,350             | 80,000            | 105,000                  | 5.2                      |
|          |                    | RT                | 114,000           | 165,000                  | 22.0                     |
|          |                    | 1,350             | 84,000            | 102,000                  | 23.0                     |
| 8        | 2,150              | 1,350             | 104,000           | 150,000                  | 16.0                     |
|          |                    | RT                | 75,000            | 99,000                   | 18.0                     |
|          |                    | 1,350             | 110,000           | 160,000                  | 25.0                     |
| 9        | 1,850              | 1,350             | 77,000            | 89,000                   | 19.0                     |
|          |                    | RT                | 105,000           | 144,000                  | 12.0                     |
|          |                    | 1,350             | 74,000            | 93,000                   | 15.0                     |
| 10       | 1,850              | 1,350             | 109,000           | 162,000                  | 23.0                     |
|          |                    | RT                | 81,000            | 95,000                   | 15.0                     |
|          |                    | 1,350             | 100,000           | 148,000                  | 15.0                     |
| 11       | 2,150              | 1,350             | 77,000            | 100,000                  | 15.0                     |
|          |                    | RT                | 168,000           | 213,000                  | 10.0                     |
|          |                    | 1,350             | 106,000           | 129,000                  | 14.0                     |

\* Specimen broke in clamp or on gauge marks.

The test results given above were obtained from specimens given the following heat treatments. Heat 1 specimens were solution treated by heating at 2000° F. for 4 hours, oil quenched and aged at 1350° F. for 24 hours and air cooled. Heat 2 specimens were heated at 1900° F. for 4 hours, oil quenched and aged at 1350° F. for 24 hours and air cooled. Heat 3 specimens were heated at 1850° F. for 1 hour, oil quenched and aged at 1350° F. for 24 hours and air cooled. Heat 4 specimens were heated at 1950° F. for 1 hour, oil quenched and aged at 1350° F. for 24 hours and air cooled. Heats 5 to 11 were solution treated by heat at the indicated temperatures for 1 hour, oil quenched and aged at 1350° F. for 24 hours and air cooled.

The following data are exemplary of the results of

these tests performed upon specimens prepared from sheet stock.

Table III

| Heat No. | Test Temp. (° F.) | Ultimate Tensile Strength (p.s.i.) | 0.2% Yield Strength (p.s.i.) | Elongation (1" gage length), Percent |
|----------|-------------------|------------------------------------|------------------------------|--------------------------------------|
| 10       | RT                | 184,500                            | 128,000                      | 18.0                                 |
|          | 1,200             | 126,100                            | 110,000                      | 20.0                                 |
|          | 1,350             | 91,500                             | 89,400                       | 29.0                                 |
| 20       | RT                | 176,400                            | 130,200                      | 16.5                                 |
|          | 1,200             | 132,300                            | 113,100                      | 16.5                                 |
| 30       | 1,350             | 101,800                            | 89,400                       | 17.5                                 |

15 The test specimens from heat 2 were cut from 0.062 inch thick sheet stock parallel to the rolling direction, heated for 20 minutes in a protective atmosphere at 1850° F., air cooled and aged at 1350° F. for 24 hours followed by air cooling. The test specimens from heat 20 3 were cut from 0.064 inch thick sheet stock transverse to the rolling direction, heated for 30 minutes in a protective atmosphere at 1900° F., air cooled and aged at 1350° F. for 24 hours, followed by air cooling.

Conventional stress rupture tests were performed upon 25 certain others of these specimens at elevated temperatures. The following data are exemplary of the results of these tests performed upon specimens prepared from bar stock.

Table IV

| Heat No. | Sol'n Temp. (° F.) | Test Temp. (° F.) | Load (p.s.i.) | Life (hrs.) | Elongation (1" gage length), Percent |
|----------|--------------------|-------------------|---------------|-------------|--------------------------------------|
| 30       | 1,350              | 1,350             | 50,000        | 307         |                                      |
|          |                    | 1,350             | 50,000        | 343         | 7.0                                  |
|          |                    | 1,200             | 90,000        | 27          | 30.0                                 |
| 40       | 1,850              | 1,200             | 85,000        | 53          | 31.0                                 |
|          |                    | 1,350             | 63,000        | 4           | 32.0                                 |
|          |                    | 1,350             | 45,000        | 47          | 43.0                                 |
| 45       | 2,000              | 1,200             | 90,000        | 229         | 12.0                                 |
|          |                    | 1,350             | 60,000        | 58          | 18.0                                 |
|          |                    | 1,350             | 55,000        | 120         | 22.0                                 |
| 50       | 1,850              | 1,350             | 45,000        | 404         | 28.0                                 |
|          |                    | 1,200             | 87,000        | 200         | 12.0                                 |
|          |                    | 1,350             | 55,000        | 124         | 12.0                                 |
| 55       | 1,850              | 1,350             | 50,000        | 129         | 19.0                                 |
|          |                    | 1,350             | 50,000        | 72          | 14.0                                 |
|          |                    | 1,200             | 90,000        | 19          | 7.2                                  |
| 60       | 1,850              | 1,350             | 50,000        | 219         | 9.3                                  |
|          |                    | 1,500             | 25,000        | 108         | 29.0                                 |
|          |                    | 1,350             | 50,000        | 75          | 32.0                                 |
| 65       | 1,850              | 1,200             | 90,000        | 101         | 8.0                                  |
|          |                    | 1,350             | 50,000        | 188         | 16.0                                 |
|          |                    | 1,500             | 25,000        | 87          | 30.0                                 |
| 70       | 1,850              | 1,350             | 50,000        | 114         | 18.0                                 |
|          |                    | 1,200             | 90,000        | 151         | 15.0                                 |
|          |                    | 1,350             | 50,000        | 231         | 15.0                                 |
| 75       | 1,850              | 1,350             | 50,000        | 102         | 28.0                                 |
|          |                    | 1,200             | 90,000        | 17          | 21.0                                 |
|          |                    | 1,350             | 50,000        | 6           | 6.7                                  |
| 80       | 2,150              | 1,350             | 50,000        | 34          | 18.0                                 |
|          |                    | 1,500             | 25,000        | 25          | 32.0                                 |
|          |                    | 1,350             | 50,000        | 53          | 24.0                                 |
| 85       | 1,850              | 1,200             | 90,000        | 178         | 8.9                                  |
|          |                    | 1,350             | 50,000        | 95          | 15.0                                 |
|          |                    | 1,500             | 25,000        | 76          | 24.0                                 |
| 90       | 2,150              | 1,350             | 50,000        | 80          | 16.0                                 |
|          |                    | 1,200             | 90,000        | 276         | 2.2                                  |
|          |                    | 1,350             | 50,000        | 316         | 3.6                                  |
| 95       | 1,850              | 1,200             | 90,000        | 181         | 13.0                                 |
|          |                    | 1,500             | 25,000        | 81          | 10.0                                 |
|          |                    | 1,350             | 50,000        | 361         | 2.4                                  |
| 100      | 2,150              | 1,200             | 90,000        | 206         | 11.0                                 |
|          |                    | 1,500             | 25,000        | 206         |                                      |

<sup>1</sup> Temperature dropped to 1,160° F. during test.

<sup>2</sup> Broke in fillet.

65 The first listed specimen in the above table from heat 1 was solution treated by heating at 2150° F. for 4 hours, oil quenched and aged at 1200° F. for 24 hours and air cooled. The second listed specimen from heat 1 was heated at 2150° F. for 4 hours, oil quenched and aged at 1350° F. for 24 hours and air cooled. The above specimens from heat 2 were heated at 1850° F. for 4 hours, oil quenched and aged at 1350° F. for 24 hours and air cooled. The above specimens from heat 3 were heated at 2000° F. for 1 hour, oil quenched and aged at 1350° F. for 24 hours and air cooled.

aged at 1350° F. for 24 hours and air cooled. The above specimens from heat 4 were heated at 2050° F. for 1 hour, oil quenched and aged at 1350° F. for 24 hours and air cooled. The above specimens from heats 5 to 11 were solution treated by heating at the indicated temperatures for one hour, oil quenched and aged at 1350° F. for 24 hours and air cooled.

The following data are exemplary of the results of these tests performed upon specimens prepared from sheet stock.

Table V

| Heat No. | Test Temp., °F. | Load (p.s.i.) | Life (hrs.) | Elongation (1/16 gage length), Percent |
|----------|-----------------|---------------|-------------|----------------------------------------|
| 2        | 1,200           | 85,000        | 305         | 17.0                                   |
|          | 1,350           | 55,000        | 29          | 37.0                                   |
| 3        | 1,200           | 90,000        | 72.5        | 9.0                                    |
|          | 1,200           | 72,000        | 1211        | -----                                  |
| 3        | 1,350           | 55,000        | 98          | 17.0                                   |
|          | 1,350           | 45,000        | 1352        | -----                                  |

<sup>1</sup> Test discontinued, specimen unbroken.

The above specimens from heat 2 were cut from 0.062 inch thick sheet stock parallel to the rolling direction and were heated in a protective atmosphere at 2000° F. for 20 minutes, air cooled and aged at 1350° F. for 24 hours followed by air cooling. The above specimens from heat 3 were cut from 0.064 inch thick sheet stock transverse to the rolling direction and were heat treated in a protective atmosphere at 2000° F. for 30 minutes, air cooled and aged at 1350° F. for 24 hours followed by air cooling.

From these and other test data, it was determined that the mechanical properties of the alloy of our invention varies to an unexpected great degree in response to quite small changes in composition and to the temperature at which the solution heat treatment is accomplished. For example, with regard to room temperature tensile properties, it will be noted that in all the heats, the highest yield and ultimate tensile strengths are attained by solution heat treating at 1850° F. Further, that while the omission of the small amounts of aluminum and zirconium produced a significant decrease in these properties in the 1850° F. solution treated material and a relatively small increase in these properties in the 2150° F. solution treated material, yet these increased room temperature yield and ultimate tensile strengths were still inferior to alloys containing these small additions and treated at 1850° F. and to the alloys without the additions which were treated at 1850° F. Similar results were obtained when the tungsten content was eliminated and also when it was significantly reduced.

When the titanium content was increased from about 2% to 3% the material solution treated at 1850° F. exhibited about a 20-30% increase in room temperature yield strength and about a 13 to 20% increase in room temperature ultimate tensile strength. The corresponding material treated at 2150° F. however did not exhibit as high an increase in these properties. When, however, the titanium content was increased to 4%, both the material solution treated at 1850° F. and the 2150° F. showed a remarkable increase in these properties.

On the other hand, much higher elevated temperature stress rupture strengths are exhibited by the alloy of our invention when the solution heat treatment is accomplished at temperatures above 1850° F. and particularly when treated at 2150° F. as shown. It will therefore be apparent that if the alloy of our invention is to be used as a structural material in high temperature environments, the optimum mechanical properties are attained by solution heat treating at about 2150° F. and aging at about 1350° F. and alloy consisting essentially of from about 30 to 35% nickel, from about 12 to 15% chromium, from about 5.5 to 7.5% tungsten, from about

5 to 5% molybdenum, from about 1.5 to 2.5% titanium, up to about 0.50% aluminum, up to about 0.50% zirconium, up to about 0.1% carbon and balance substantially all iron with no more than the previously noted amounts of impurities. If, however, high room temperature mechanical properties are desired, the titanium content of the alloy should be increased to the range 2.5 to about 4.5% titanium and the solution heat treatment should be decreased to about 1850° F. and the material aged at about 1350° F.

As shown, it may therefore be seen that the alloy of our invention, at room temperature, exhibits an ultimate tensile strength of up to about 220,000 p.s.i. or higher, a 0.2 percent offset yield strength of about 190,000 p.s.i. or higher, and the ductility is from about 3.5 to 24 percent elongation. At 1350° F. the ultimate tensile strength is up to about 129,000 p.s.i. the 0.2 percent offset yield strength is about 100,000 p.s.i. or higher, and the ductility is from about 1 to 25 percent elongation.

15 The stress rupture tests indicate by extrapolation that the alloys of our invention will withstand a continuously applied load of about 76,000 p.s.i. for 1000 hours at 1200° F. and a continuously applied load of about 41,000 p.s.i. for 1000 hours at 1350° F. before fracturing.

20 In comparison with previously known alloys having similar compositions, one such commercially available alloy having the composition of about 44 percent nickel, 34.5 percent iron, 12.8 percent chromium, 5.7 percent molybdenum, 2.4 percent titanium, 0.45 percent manganese, 0.23 percent silicon, 0.03 percent copper, 0.01 percent sulfur, and 0.04 percent carbon has been found to have the following mechanical properties.

Table VI

|    | Testing Temperatures (° F.) |           |           |
|----|-----------------------------|-----------|-----------|
|    | Room Temp.                  | 1,200° F. | 1,350° F. |
| 40 | Ult. Tens. Str.-----p.s.i.  | 174,000   | 135,000   |
|    | 0.2% Yield Str.-----p.s.i.  | 102,000   | 98,000    |
|    | Percent Elongation-----%    | 19        | 20        |
|    |                             |           | 102,000   |
|    |                             |           | 82,000    |
|    |                             |           | 11        |

45 Bar stock specimens of this material have been found to have a 1000 hour stress rupture strength of about 55,000 p.s.i. at 1200° F., and a 1000 hour stress rupture strength of about 30,000 p.s.i. at 1350° F.

50 Another similar commercially available alloy consisting essentially of 26 percent nickel, 15 percent chromium, 1.5 percent molybdenum, 1.6 percent titanium, 0.17 percent aluminum, 0.2 percent vanadium, 0.05 percent carbon, and the balance substantially all iron, has been found to have the following mechanical properties.

Table VII

|    | Testing Temperatures (° F.) |           |           |
|----|-----------------------------|-----------|-----------|
|    | Room Temp.                  | 1,200° F. | 1,350° F. |
| 60 | Ult. Tens. Str.-----p.s.i.  | 157,000   | 110,000   |
|    | 0.2% Yield Str.-----p.s.i.  | 98,000    | 93,000    |
|    | Percent Elongation-----%    | 25        | 10        |
|    |                             |           | 74,000    |
|    |                             |           | 68,000    |
|    |                             |           | 10        |

65 Bar stock specimens of this material have been found to have a 1000 hour stress rupture strength of about 50,000 p.s.i. at 1200° F. and a 1000 hour stress rupture strength of about 23,000 p.s.i. at 1350° F.

70 From the foregoing it is apparent that the alloy of our invention has mechanical properties which are superior to previously known comparable alloys. Further, the alloy of our invention retains its strength at elevated temperatures to a greater degree than such previously known materials. The alloy of our invention is readily formable into sheet stock and is readily welded, the

welded joints retaining their strength and ductility. In addition, being austenitic, the alloy of our invention is highly resistant to corrosion at elevated temperatures.

While we have discussed certain specific heat treating schedules in the foregoing specification for purposes of rendering a more complete disclosure, we do not wish our invention to be limited to any particular treatment or composition except as defined in the appended claims.

What we claim as new and desire to secure by Letters Patent of the United States is:

1. An alloy consisting essentially of from about 30 to 35 percent by weight nickel, from about 12 to 15 percent chromium, from about 5.5 to 7.5 percent tungsten, from about 2.5 to 5.0 percent molybdenum, from about 1.5 to 4.5 percent titanium, up to about 0.50 percent aluminum, from 0.01 to about 0.50 percent zirconium, up to about 0.10 percent carbon and the balance substantially all iron.

2. An alloy consisting essentially of from about 31.0 to 34 percent by weight nickel, about 12.5 to 15.0 percent chromium, about 6.0 to 7.0 percent tungsten, about 3.0 to 4.6 percent molybdenum, about 1.50 to 2.5 percent titanium, about 0.2 to 0.5 percent aluminum, from 0.01 to about 0.4 percent zirconium, not more than 0.08 percent carbon, balance substantially all iron and no more 20

than 0.2 total weight percent of manganese, silicon, sulfur and phosphorus.

3. An alloy consisting essentially of about 33 percent by weight nickel, about 13 percent chromium, about 6.5 percent tungsten, about 3.5 percent molybdenum, about 2.0 percent titanium, about 0.45 percent aluminum, about 0.35 percent zirconium, less than about 0.08 percent carbon, not more than about 0.05 percent manganese, not more than about 0.05 percent silicon, not more than about 0.04 percent 10 sulfur, not more than about 0.04 percent phosphorus and the balance substantially all iron.

4. An alloy consisting essentially of from about 31 to 34% by weight nickel, about 12.5 to 15.0% chromium, about 6.0 to 7.0% tungsten, about 3.0 to 4.6% molybdenum, about 2.5 to 4.5% titanium, about 0.2 to 0.5% aluminum, from 0.01 to about 0.4% zirconium, not more than 0.08% carbon, balance substantially all iron and no more than 0.2 total weight percent of manganese, silicon, sulfur and phosphorus.

References Cited in the file of this patent

UNITED STATES PATENTS

2,047,916 Lohr \_\_\_\_\_ July 14, 1936  
2,432,617 Franks et al. \_\_\_\_\_ Dec. 16, 1947